

April 23, 1963

K. SIEBERTZ

3,086,856

METHOD AND DEVICE FOR THE SUCCESSIVE ZONE  
MELTING AND RESOLIDIFYING OF  
EXTREMELY PURE SUBSTANCES

Filed Feb. 10, 1954

FIG.1



FIG.4



FIG.2



FIG.3



# United States Patent Office

3,086,856

Patented Apr. 23, 1963

1

3,086,856

## METHOD AND DEVICE FOR THE SUCCESSIVE ZONE MELTING AND RESOLIDIFYING OF EXTREMELY PURE SUBSTANCES

Karl Siebertz, Munich, Germany, assignor to Siemens & Halske Aktiengesellschaft, Berlin and Munich, Germany, a German corporation

Filed Feb. 10, 1954, Ser. No. 409,420

Claims priority, application Germany Feb. 14, 1953  
6 Claims. (Cl. 75—10)

It is known to liberate last traces of impurities from generally pure materials by successively melting a zone of an elongated body or rod of the material in such a manner that the molten zone travels gradually from one end of the body to the other. Due to the concentration jump of the dissolved impurities in the border surface between the liquid and solid portions of the rod, the molten zone becomes enriched in impurities while a depletion occurs in the resolidifying material, or vice versa. Due to the fact that the melting zone is gradually displaced from one to the other end of the rod, the impurities also migrate toward one of these ends. If necessary, the process can be repeated for obtaining maximum degrees of purity. At the same time, the process may serve to produce a single crystal from an originally amorphous or polycrystalline material, which may be sintered or otherwise produced. This requires placing into the melting zone, at the point where it commences its travel along the body, a single crystal of the proper orientation to serve as a crystal germ.

The zone-melting process as heretofore known requires placing the material to be melted into a crucible or boat of refractory material. The results of the process, therefore, are affected by the fact that the material being processed can take up new impurities from the surface of the crucible walls.

It is an object of my invention to avoid this deficiency and to improve the zone-melting method toward achieving a higher degree of purity of the material being treated and toward a reduction in the processing time needed for securing a given degree of purity.

To this end, and in accordance with a feature of my invention, the body to be successively zone melted is mechanically supported at only a few places so that the melting zones are only in the slightest degree, if at all, in contact with the means holding or containing the body. To prevent the molten material from running off due to its gravity, the melting zone is kept so narrow that the surface tension suffices for retaining it between the adjacent solid parts of the material. To achieve this result, and according to another feature of my invention, the elongated and preferably rod-shaped body is arranged vertically, in contrast to the horizontal arrangement heretofore customary.

According to another feature of my invention, the running-off of the molten material is prevented by continuously revolving the body during the zone-melting operation.

According to still another feature of the invention, the body may be given a horizontal or inclined arrangement and is heated only from above so that the melting zone does not extend through the entire diameter of the rod but forms only a molten segment or cone-shaped zone comprising only about the upper half of the rod, while the lower part of the rod remains solid and carries the melting zone.

According to a further feature of the invention, the liquid material in the melting zone, which in this case may traverse the entire cross section of the rod, is kept freely floating by electromagnetic or pneumatic means. To this end, an electric field may be produced which, at

2

the place of the melting zone, produces potential surfaces of a corresponding shape, for instance saddle shape, to magnetically support the material, the material being electrically conductive at least when in its molten condition. The same effect can be obtained by the coaction of correspondingly arranged streams of gas. The gas to be used for this purpose is the same protective or inert gas that forms the atmosphere within which the entire zone-melting operation is to be performed.

10 The foregoing and other features of the invention will be more fully understood from the following description of the embodiments of devices according to the invention illustrated on the drawing, in which—

15 FIG. 1 illustrates an arrangement for heat-treating a vertically held elongated body of material according to the invention wherein the melted zone is prevented from running off by means of a plurality of inclined blowers;

20 FIG. 2 illustrates an alternative method of practicing the invention wherein the material being treated is horizontally or slantingly disposed;

25 FIG. 3 is a transverse cross-sectional view of FIG. 2 taken through the melted zone; and

FIG. 4 shows an apparatus for performing the method according to the invention with an arrangement as shown

25 in FIG. 1.

According to FIG. 1, a rod 1, of aluminum for example, to be processed is held in vertical position by clamping devices 2 and 3 engaging the two ends of the rod. A directly or indirectly heated ring 4 of small axial width 30 in comparison with the length of the rod 1 surrounds a zone 5 of the rod in concentric relation thereto. The whole device is located in a vacuum or within a protective inert gaseous medium. A number of nozzles 6 are distributed around the rod below the heater 4. Their 35 blowing direction is such that the melting zone 5 is impinged on all sides from below so that the molten material cannot drop off. The gas supplied to the nozzle 6 is preheated by a heating device (not shown) to prevent marginal cooling of the melting zone. The clamps 2 and 3 together with the rod 1 are displaceable in the direction of the arrow 7 relative to the stationarily mounted heating and blowing devices 4, 6. The mechanism for moving the holders together with the rod may 40 comprise a motor driven worm screw, a guide device for allowing simultaneous translatory motion of the two holders, and gear mechanism carried by the holders and in meshing engagement with the worm screw. During the operation, therefore, the melting zone 5 travels from the bottom upwardly along the rod.

50 In the embodiment shown in FIGS. 2 and 3, the rod 1 of the material to be purified is arranged horizontally. An arc lamp 8 serves as a source of heat. Its radiation is concentrated upon the surface of rod 1 by means of a hollow mirror 9 and produces a trough or cone-shaped melting zone 10. This melting zone is carried by the underlying solid portion of the rod. A blowing device 11 directs a cooling stream of protective gas against the bottom side of rod 1 to prevent the melting zone from breaking through the solid area. The rod 1 is continuously kept in revolution in the direction of the arrow 12

60 by means of a motor (not illustrated) adapted to turn a holding device at one end of the rod being processed. In addition, the radiation source 8, 9 is displaced relative to rod 1 in the direction of the arrow 13. This can be 65 accomplished by having the heat source and blowers fixed on a support that is slideable in guide means coextensive with the rod, and by providing a motor of suitable speed having an output shaft cooperatively connected with the displaceable support. As a result, the melting zone 10 is drawn through the rod from the left to the right on a helical path. FIG. 3 shows the heating and cooling means in relation to a cross section of rod

1 through the melting zone 10. As apparent from FIG. 3, the heat source 8, 9 is given a somewhat slanting arrangement while the cooling effect of the nozzle arrangement 11 extends over a larger peripheral range of the rod and is effective not only from below but also from the side of the rod.

In the device according to FIG. 4, the rod 1 to be processed is mounted at both ends in respective holders 2, 3 and is surrounded by a ring-shaped heater 4 for melting an axially narrow cross-sectional zone 5 as described above with reference to FIG. 1. Holder 3 is mounted on a support 21 which is slidably connected with a base plate 22 and can be displaced in the axial direction of rod 1 by means of a screw spindle 23. A bell-shaped housing 24 sealed against the base plate 22 encloses the rod 1 to permit operating in vacuum or in a protective atmosphere. The holder 2 is mounted on a shaft 25 that passes through the housing to the outside and carries a gear 26 to be driven from a motor 27. The heater ring 4 is mounted on an axially displaceable rod 28 that extends to the outside of the housing 24 where it is connected by a rope 29 with a reel 30.

Operating the reel, for instance by means of another motor, causes the rod 28 and the heater 4 to progress along the rod 1, for instance, in the direction of the arrow 7 for zone-melting the rod in the manner described. During the processing, the spacing between the holders 2 and 3 can be varied for controlling the cross section of the processed portion of material. Also during the zone-melting, the motor 27 may be operated to keep the upper portion of rod 1 in revolution. If desired, another motor may be provided for also revolving the holder 3 with the lower portion of rod 1.

A magnet coil 31 is mounted on rod 28 in concentric relation to heater ring 4 to produce during the melting operation a magnetic field to counteract the tendency of the molten material to run off. For the same purpose the device is also equipped with the above-described nozzles 6 that, when in use, blow a stream of gas upwardly against the molten zone. The gas may be identical with the one used as a protective atmosphere. The nozzles are preferably mounted together with the heater so that they maintain, during the travel motion, their proper spacing from the molten zone.

I claim:

1. The process of successively zone-melting and re-solidifying a rod of fusible material which comprises supporting said rod at opposite end portions in a vertical position, applying heat to establish a molten segmental zone extending only part way across the cross section of the rod, the axial width and cross-sectional area of said molten zone being such that the amount of molten material is limited to that which is supportable solely by virtue of cohesive and adhesive forces, and displacing said molten zone in an axial direction along said rod, while at the same time turning said rod so that substantially all surface portions thereof are progressively melted,

4  
the molten zone moving in a helical path in and along said body.

2. The process of claim 1, the molten segmental zone extending not more than half way across the cross section of said rod.

3. The process of successively zone-melting and re-solidifying a rod of fusible material which comprises supporting said rod at opposite end portions, applying heat to establish a molten segmental zone extending only part way across the cross section of the rod, the axial width and cross-sectional area of said molten zone being such that the amount of molten material is limited to that which is supportable solely by virtue of cohesive and adhesive forces, and displacing said molten zone in an axial direction along said rod, while at the same time turning said rod so that substantially all surface portions thereof are progressively melted, the molten zone moving in a helical path in and along said body.

4. The process of claim 3, the molten segmental zone extending not more than half way across the cross section of said rod.

5. The method of processing an elongated rod-shaped body of meltable material of delimited length, comprising clampingly supporting the body at opposite end portions, 25 heating a segmental zone of said body to molten temperature, said zone extending only part way across said body, and advancing said heating along said body, the axial length and cross-sectional area of said molten zone being small enough so that surface tension serves to contain said molten zone in position along said body.

6. The crucible-free method of zone-melting an elongated rod-shaped body of meltable material, comprising supporting the body at its end regions, heating a transversely extending zone of said body to molten temperature, the zone extending at least part way across said body, advancing said molten zone lengthwise along said rod-shaped body, while directing a blast of preheated inert gas so that it impinges against the molten zone, serving to counteract gravitational force acting on the molten material by preventing the dropping off of molten material, and also serving to prevent marginal cooling of the melting zone.

#### References Cited in the file of this patent

#### UNITED STATES PATENTS

|           |                  |               |
|-----------|------------------|---------------|
| 2,254,306 | Mott et al.      | Sept. 2, 1941 |
| 2,683,676 | Little et al.    | July 13, 1954 |
| 2,686,864 | Wroughton et al. | Aug. 17, 1954 |
| 2,739,088 | Pfann            | Mar. 20, 1956 |
| 3,030,194 | Emeis            | Apr. 17, 1962 |

#### FOREIGN PATENTS

|           |        |               |
|-----------|--------|---------------|
| 1,065,523 | France | Jan. 13, 1954 |
| 1,087,946 | France | Sept. 1, 1954 |

#### OTHER REFERENCES

Keck and Golay: Phys. Rev. 89, 1297 (1953).